

1

3,623,864

### MACHINABLE ALLOY

George A. Majesko, Glen Ridge, N.J., assignor to  
Wilbur B. Driver Company  
No Drawing. Filed Apr. 13, 1970, Ser. No. 28,045  
Int. Cl. C22c 19/00

U.S. CL. 75—170

3 Claims

### ABSTRACT OF THE DISCLOSURE

A freely machinable alloy comprising, as expressed in percent by weight:

Nickel: 50.0%—52.0%

Selenium: 0.1%—0.4%

Manganese: 0.5%—2.0%

Iron: Balance

### CROSS REFERENCE TO RELATED APPLICATIONS

In co-pending patent application S.N. 873,508, filed Nov. 3, 1969, selenium additions to different alloys, namely iron-nickel-cobalt alloys, are disclosed by the same inventor and assigned to the same assignee as the present application. The alloys contemplated herein are nickel-iron-alloys.

### SUMMARY OF THE INVENTION

Certain alloys of the nickel-iron type are used in forming seals between metals and glass or metals and ceramics as well as in other applications wherein the thermal coefficients of expansion and other properties are critical.

These alloys are characterized by the undesirable property of poor machinability. As a result, tools used in shaping such alloys wear much too rapidly, even when the machining is carried out at relatively low speeds and feed rates.

I have discovered that the addition of selenium in amounts falling within the range 0.1% to 0.4% (by weight) coupled with the simultaneous addition of manganese in amounts falling within the range 0.5%—2.0% to a nickel-iron alloy comprising 50%—52% nickel, balance iron, results in alloys with sharply enhanced machinability and, at the same time, with otherwise substantially unchanged physical and mechanical properties. As a result, excessive tool wear no longer takes place.

### DETAILED DESCRIPTION OF PREFERRED EMBODIMENTS

A first plurality of alloys were fabricated with compositions falling within the ranges set below:

Nickel: 50.0%—52.0%

Selenium: 0.1%—0.4%

Manganese 0.5%—2.0%

Minor elements (silicon, carbon, etc.): 1%

Iron: Balance

A second plurality of alloys without selenium and with a manganese content of less than 0.5% but otherwise of like composition to the first plurality were fabricated in the same manner.

Both sets of alloys were tested for machinability in ac-

2

cordance with the different r.p.m. and feed rates set forth in Table I below:

TABLE I

|    | Diameter in inches | r.p.m. | Feed rate, inches/rev. | Surface, feet/minute |
|----|--------------------|--------|------------------------|----------------------|
| 5  | .750               | 280    | .0042                  | 55                   |
|    | .725               | 380    | .0042                  | 72                   |
|    | .700               | 510    | .0042                  | 93                   |
|    | .680               | 665    | .0042                  | 113                  |
|    | .650               | 867    | .0042                  | 142                  |
| 10 | .600               | 1,185  | .0042                  | 186                  |
|    | .575               | 1,600  | .0042                  | 241                  |
|    | .550               | 1,600  | .0060                  | 230                  |
|    | .525               | 1,600  | .0077                  | 219                  |
|    | .500               | 1,600  | .0096                  | 209                  |
|    | .475               | 1,600  | .0135                  | 199                  |
|    | .450               | 1,600  | .0170                  | 188                  |
| 15 | .425               | 1,600  | .0237                  | 178                  |
|    | .400               | 1,600  | .0288                  | 167                  |
|    | .375               | 1,600  | .0340                  | 157                  |
|    | .350               | 1,600  | .0384                  | 147                  |

For constant depth of cut (.025") and feed rate (.0042 inches/rev.) the selenium-containing alloys could be turned on a lathe at 241 surface feet per minute with no undesirable effects. The work piece remained cool. The selenium free alloys became very hot at 72 surface feet per minute and the machining lubricant began to smoke at 93 surface feet per minute causing a sharp deterioration of the surface finish.

At a constant r.p.m. of 1600 and a depth of cut of .025", the selenium containing alloys could be fed in a trouble free manner at rates ranging from .0042 to .0384 inches/rev. Under the same conditions the selenium-free alloys ruined the tool when the feed rate was increased beyond .0060 inches/rev.

I found that when the selenium content was reduced below about 1% and the manganese content was reduced simultaneously below 0.5%, the machinability characteristics were not substantially improved as compared to known alloys. When the selenium content was increased about 0.4% and the manganese content was increased simultaneously above 2.0%, the machinability characteristics were not degraded, but the thermal expansion properties of the alloys began to vary beyond the ranges specified and required. As long as the selenium and manganese additions are maintained within the ranges set forth herein, any increase of selenium content must be accompanied by an increase (not necessarily a proportional increase) in the manganese content to maintain forgeability.

What is claimed is:

1. A freely machinable alloy consisting essentially of, as expressed in percent by weight:

Nickel: 50.0%—52.0%

Selenium: 0.1%—0.4%

Manganese: 0.5%—2.0%

Iron: Balance

2. An alloy as set forth in claim 1 wherein any increase of selenium content within 0.1%—0.4% must be accompanied by an increase of manganese content within the range of 0.5%—2.0%.

3. An alloy as set forth in claim 2 containing less than 1% of minor elements such as silicon and carbon.

### References Cited

| UNITED STATES PATENTS |           |        |             |        |
|-----------------------|-----------|--------|-------------|--------|
| 65                    | 2,471,079 | 5/1949 | Post et al. | 75—170 |
|                       | 3,138,454 | 6/1964 | Williams    | 75—170 |

RICHARD O. DEAN, Primary Examiner